

## 1

3,189,449

**COLLOID STRATUM TRANSFER PROCESS**  
 Richard G. Yost, Rochester, N.Y., assignor to Eastman  
 Kodak Company, Rochester, N.Y., a corporation of  
 New Jersey  
 No Drawing. Filed Oct. 1, 1962, Ser. No. 227,562  
 4 Claims. (Cl. 96—28)

This invention concerns an activator for use with the photographic process known as the colloid transfer process.

In the colloid transfer process, an image in soft adhesive organic colloid is formed photographically and a discrete stratum of the image is transferred to a receiving sheet to provide a reproduction of the subject. The process is described in the Yutzy et al. U.S. Patents 2,596,756, granted May 3, 1952, and 2,716,059, granted August 23, 1955, and embodies the exposure to a subject of substantially unhardened gelatino-silver halide emulsion layer which may contain a gelatin tanning silver halide developing agent as well as a non-tanning silver halide developing agent.

Upon activation of the exposed gelatin emulsion with the alkaline solution in the presence of the developing agent or agents, tanning development of the most exposed regions of the emulsion corresponding to the highlights of the subject proceeds, although some development of the less exposed regions also takes place to provide visual density for the transferred image as explained in more detail in U.S. Patent 2,716,059 above. Thereafter, the developed emulsion is pressed into contact with an absorbent receiving sheet such as paper to cause the less exposed regions, and thus the less developed regions, of the emulsion to adhere to the receiving sheet. Subsequently, when the emulsion and receiving sheet are separated, a stratum of the less exposed regions of the emulsion remains on the sheet and appears as a positive silver image of the original subject.

As mentioned in the above patents, the alkaline solution used for activation of the exposed emulsion layer advantageously contains a gelatin softening agent to facilitate transfer of the less exposed portions of the emulsion to the receiving sheet. Urea and certain other gelatin softening agents have been suggested for this purpose. The above patents also suggest the use of sodium carbonate as the alkaline component of the alkaline solution used for initiating development of the exposed emulsion.

In one embodiment of the colloid transfer process, it has been proposed that the process become more automated and that the time for obtaining a copy be shortened. For this reason, it has been desirable to have an activator which would decrease the activation time formerly used and permit more rapid processing than the 15 to 20 second period normally required with known activators. In addition, certain advantages over the older activators have been sought. For instance, temperature has normally had to be regulated requiring a thermostated temperature control to keep the system at satisfactory working conditions. Therefore, it was desirable to find an activator solution which could be used between the temperatures of 60 to 90° F. without temperature regulation between these limits.

It was also desirable to increase the number of transfer matrices with a given amount of activator solution and to have a solution that is stable for long periods in liquid form.

I have found an activator solution which can be used at room temperature containing tripotassium phosphate, potassium salicylate, and other additives such as sequestering agents, anti-foamants, and the like.

One object of this invention is to provide an improved

## 2

colloid transfer activator solution having a useful temperature range of 60–90° F. Another object is to provide an improved activator solution which has a high capacity, good stability and high speed. Another object is to provide a method of preparing an activator solution which has improved characteristics. A further object is to provide a method of processing an exposed matrix for use in the colloid transfer system using an improved activator solution. Additional objects will be apparent from the following disclosure.

The above objects are attained by using an activator solution having the following components:

|                                                  | Grams/liter |
|--------------------------------------------------|-------------|
| 15 Tripotassium phosphate                        | 60–90       |
| 15 Potassium salicylate                          | 10–40       |
| 15 Ethylenediamine tetraacetic acid, sodium salt | 0–10        |
| 15 Tetraethyleneglycol                           | 0–40        |
| Water to make 1 liter.                           |             |

The pH of the above activator solution is approximately 20 12.3 at 70° F. and the solution activates satisfactorily down to a pH of about 11.3.

The solution can be prepared from equivalent amounts of, for example, potassium hydroxide, phosphoric acid, and salicylic acid instead of the salts.

25 Anti-foam agents may be used, particularly in the event that the activator is to be used in a mechanical agitating device.

The following examples are intended to illustrate my invention but not to limit it in any way.

## Example 1

An activator for the colloid transfer process is prepared by dissolving 80 grams of tripotassium phosphate in 800 ml. of water; 20 grams of potassium salicylate is added with stirring. Forty milliliters of tetraethyleneglycol and 5 grams of ethylenediamine tetraacetic acid tetrasodium salt are dissolved before bringing the volume to 1 liter.

The activator as prepared above is used in a colloid transfer process of the type described in Yutzy et al. U.S. Patent 2,596,756. When the exposed matrix is soaked for 6 seconds and pressed in contact with a receiving sheet, a good quality image is obtained by transfer in the unexposed areas. The temperature of the activator is 45 80° F. When the temperature is varied over a 60–90° F. range, satisfactory transfers are obtained producing good clear images over the entire temperature range.

A tray containing 1 liter of the above activator is used to process a series of matrices. Successive copies are 50 made until 240 sheets have been soaked and transferred, when due to loss of solution activity, the images are no longer of acceptable quality.

## Example 2

55 An activator solution is prepared as in Example 1, except the amount of tripotassium phosphate is varied between 60 and 100 grams. Within this range satisfactory transfers are obtained. Where less than 60 grams of tripotassium phosphate are used, the matrix becomes 60 too soft for satisfactory use. When more than 100 grams of tripotassium phosphate are used, very little transfer takes place and on standing an undesirable degree of crystal growth takes place at the edges of the tray.

## Example 3

An activator of the following composition is prepared:

|                                                       | Grams |
|-------------------------------------------------------|-------|
| 70 Tripotassium phosphate                             | 80    |
| 70 Potassium salicylate                               | 10    |
| 70 Ethylenediamine tetraacetic acid, tetrasodium salt | 5     |
| 70 Tetraethyleneglycol                                | 40    |

When this solution is used to activate a colloid transfer matrix for 6 seconds at 75° F., very good transfers are made. When the potassium salicylate is increased to 40 grams/liter, satisfactory transfers are also obtained.

*Example 4*

An activator is prepared having the following composition:

|                                                    | Grams |
|----------------------------------------------------|-------|
| Tripotassium phosphate                             | 80    |
| Potassium salicylate                               | 20    |
| Ethylenediamine tetraacetic acid, tetrasodium salt | 5     |

Copies are made with a 6-second activation time. However, on standing for extended periods, an excess amount of crystallization occurs on the transfer mechanism which prevents satisfactory contact and transfer for subsequent use of the activator.

*Example 5*

The following composition is prepared:

|                                                    | Grams |
|----------------------------------------------------|-------|
| Tripotassium phosphate                             | 80    |
| Urea                                               | 20    |
| Ethylenediamine tetraacetic acid, tetrasodium salt | 5     |
| Volume to 1 liter.                                 |       |

The above activator works satisfactorily in the transfer process when it is freshly prepared. However, after 6 months storage at 80° F., the activator fails to produce softening action so that images can not be transferred to the receiving sheet. Therefore, it would be impractical to store such a solution for extended periods before use and use within a short time would be required to obtain good results.

*Example 6*

An activator solution is prepared having the following proportions. 75 grams of trisodium phosphate are dissolved in 800 ml. of water and 25 grams of sodium salicylate are dissolved in the solution. 5 grams of ethylenediamine tetraacetic acid, tetrasodium salt and 40 ml. of tetraethylene glycol are added with water to bring the solution to 1 liter. On soaking at room temperature for 6 seconds, a transfer which had good sharpness and high quality is made to the receiving sheet. When the solution is permitted to remain in the tray for about two days, crystals begin to grow at the edge and on exposed wet surfaces, which interfere with normal operating procedure.

*Example 7*

A substantially unhardened gelatin-silver halide emulsion (having a hardness as defined in the above patents) is prepared as described in U.S. Patent 2,716,059 above and containing a mixture of tanning and substantially non-tanning silver halide developing agents such as 4-phenylcatechol and 4-methoxy- $\alpha$ -naphthol. The emulsion is coated on a paper support and dried. The resultant sensitive element is then exposed to a two-tone subject (a line or halftone subject) if desired by reflex methods, and placed in the following alkaline solution of the invention to initiate development:

|                        | Grams |
|------------------------|-------|
| Tripotassium phosphate | 80    |
| Sodium salicylate      | 30    |
| Water to make 1 liter. |       |

When hard waters are used in making up the above solution, in order to prevent the formation of scale on equipment it is advisable to add a water softening agent, such as well known alkaline earth metal chelating agents, e.g., ethylenediamine tetraacetic acid, di- or tetrasodium salts, isopropanoldiaminetetraacetic acid salts, etc. About 5 grams of the salts are useful in the above formula for this purpose.

While development in the above alkaline solution is proceeding, light should be excluded to the extent re-

quired by the particular silver halide present in the emulsion. With daylight working emulsions limited exposure to room lights may be given during the exposure and development steps. Other emulsions may require the use of the usual safelights during the exposure and processing steps. When the proper amount of exposure has been given, gelatin tanning silver halide development occurs principally in the more highly exposed areas of the emulsion and little or no tanning development in the other areas.

When development is complete as determined by trial with the particular emulsion and conditions of operation in use, the sensitive element is pressed into contact with an absorbent sheet such as paper by means of a squeegee blade or rollers. Immediately thereafter, the sensitive element and receiving sheet are separated leaving a stratum of the less exposed and thus less hardened regions of the emulsion adhered to the receiving sheet. The result is a positive line or halftone silver-containing image affixed to the sheet.

The reception sheet for the process is advantageously prepared as described in the Chan et al., U.S. Patent 2,865,745, issued December 23, 1958, comprising a paper sheet on the surface of which is a mixture of an intensifying agent such as thiourea and a development suppressing agent, such as sodium formaldehyde bisulfite.

The quantity of sodium salicylate and tripotassium phosphate in the alkaline solution may be varied from that given in the above formula depending upon the requirements of the particular emulsion used in the process. However, the emulsion should have a maximum hardness of the order mentioned by the above patents corresponding to a gelatin layer containing about 0.7 gram of dry formaldehyde per pound of gelatin freshly coated. For instance, the optimum amount of tripotassium phosphate may be readily determined by experiment with different emulsions, development times, and temperatures. Since the tripotassium phosphate furnishes the alkaline component of the solution, development is accelerated by use of higher amounts and conversely slowed by lower amounts.

In a preferred embodiment of the invention the gelatin tanning and non-tanning developing agents are present in the emulsion. However, either or both developing agents may be present in the alkaline solution and the other in the emulsion. A very useful combination of developing agents is 4-phenylcatechol with 4-methoxy- $\alpha$ -naphthol. Since the latter is self-coupling, it forms a colored compound during development which contributes density to the print. Other useful tanning and non-tanning silver halide developing agents are disclosed by the above patents.

The proportions used in this activator solution are critical within the limits given above. For instance, if the concentration of the tripotassium phosphate is over 100 grams/liter, transfer is difficult and excessive crystallization will occur upon evaporation. If the concentration is below 60 grams/liter, the solution has a reduced useful life.

It will be appreciated that the sequestering agent can be some other agent than ethylenediamine tetraacetic acid tetrasodium salt providing that it effectively sequesters calcium or other hardness cations in water used to make or dilute the activator solution. The amount of anti-foam agent would depend upon the conditions, such as pumping or agitating operations which may tend to generate foam. This amount can be judged effectively by one skilled in the art.

I claim:

1. A method of photographic reproduction which comprises developing an exposed, substantially non-hardened, gelatin-silver halide emulsion layer, said emulsion being not harder than a gelatin layer containing 0.7 gram of formaldehyde per pound of gelatin freshly coated, with a solution of tripotassium phosphate and potassium salicy-

late in the presence of both a gelatin tanning silver halide developing agent and a substantially non-tanning silver halide developing agent to obtain a hardened gelatin and silver image in the areas of the emulsion layer corresponding to the highlights of the subject, and substantially unhardened gelatin, silver, and silver halide in the areas of the emulsion layer corresponding to the shadows of the subject, said development being such as to prevent any substantial tanning of the emulsion layer in said areas corresponding to the shadows of the subject, pressing a sheet having an absorbent surface against said emulsion layer while said emulsion layer is moist to cause only the shadow areas of the emulsion to adhere to the sheet, and separating said sheet and emulsion layer to transfer only a stratum of said shadow areas of the emulsion layer to said sheet.

2. The process of claim 1 wherein the gelatin tanning silver halide developing agent and the substantially non-tanning silver halide developing agent are present in the emulsion layer before exposure.

3. A method of photographic reproduction which comprises developing an exposed, substantially non-hardened gelatino-silver halide emulsion layer, said emulsion being not harder than a gelatin layer containing 0.7 gram of formaldehyde per pound of gelatin freshly coated, with a solution comprising 60-90 grams/liter of potassium phosphate, 0-10 grams/liter sequestering agent, 10-40 grams/liter potassium salicylate, 0-40 grams/liter tetrachylene glycol and water in the presence of both a tanning silver halide developing agent and a substantially non-tanning silver halide developing agent.

liter potassium salicylate, 0-40 grams/liter tetrachylene glycol and water in the presence of both a tanning silver halide developing agent and a substantially non-tanning silver halide developing agent.

4. The process of claim 3 wherein the gelatin tanning silver halide developing agent and the substantially non-tanning silver halide developing agent are present in the emulsion layer before exposure.

|    |                                  |      |                            |
|----|----------------------------------|------|----------------------------|
| 10 | References Cited by the Examiner |      |                            |
|    | UNITED STATES PATENTS            |      |                            |
|    | 2,156,626                        | 5/39 | Ham ----- 96-66            |
|    | 2,384,592                        | 9/45 | Bean ----- 96-66           |
|    | 2,596,756                        | 5/52 | Yutzy et al. ----- 90-28   |
| 15 | 2,625,476                        | 1/53 | Henn ----- 96-66           |
|    | 2,716,059                        | 8/55 | Yutzy et al. ----- 96-28   |
|    | 2,834,676                        | 5/58 | Stanley et al. ----- 96-66 |
|    | 3,043,687                        | 7/62 | Linge ----- 96-28          |

|    |                  |                                                                |  |
|----|------------------|----------------------------------------------------------------|--|
| 20 | OTHER REFERENCES |                                                                |  |
|    | Mees:            | The Theory of the Photographic Process, 1942,<br>p. 391.       |  |
| 25 | Rose:            | The Condensed Chemical Dictionary, 5th ed.,<br>1956, page 898. |  |

NORMAN G. TORCHIN, Primary Examiner.